

## UNITED STATES PATENT OFFICE

1,975,376

## ALLOY

Georg Schichtel, Dobrach - on - Millstattersee,  
Austria, assignor to American Magnesium  
Metals Corporation, Pittsburgh, Pa., a corpo-  
ration of Delaware

No Drawing. Original application February 14,  
1933, Serial No. 656,765. Divided and this ap-  
plication August 22, 1933, Serial No. 686,320.  
In Austria February 19, 1932

3 Claims. (Cl. 75—1)

This application is a division of my prior ap-  
plication Serial No. 656,765 filed February 14,  
1933.

The present improved alloy is one in which  
5 magnesium is the predominant element, the pri-  
mary object being to develop an alloy that will  
possess the characteristic low specific gravity  
which is obtained by the use of magnesium in ex-  
cess of 80 per cent while such alloy will be char-  
acterized by higher resistance to corrosion and at  
10 the same time will have a higher strength than  
the known alloys of this kind.

The known alloys in use containing generally  
more than 85% magnesium and as principal ad-  
ditional ingredient aluminum or zinc or both of  
15 these ingredients, other constituents such as man-  
ganese being present in relatively small amounts,  
do not exhibit a sufficient resistance to corrosion  
by water or even by damp air, and cannot be used  
20 at all when in continuous contact with sea-water.  
Various attempts have been made to render the  
surfaces of these metals more resistant by apply-  
ing coatings, but such attempts failed since cor-  
rosion often takes place to an increased extent  
25 when the superficial protective layer is damaged.

The object of the invention is attained by the  
addition of further additional metals to the  
alloys, namely antimony or bismuth or both of  
30 these metals amounting in general to not less than  
0,05% and not more than 2% of the total.

The most diverse alloys of the kind referred to  
containing antimony or bismuth have proved dis-  
tinctly superior, when exposed to the action of a  
35 3% solution of common salt, to alloys of the same  
kind which do not contain antimony or bismuth;  
whilst the alloys containing antimony or bis-  
muth showed an almost unaltered surface, the  
samples devoid of antimony or bismuth were  
40 strongly corroded on carrying out the compara-  
tive tests.

In general the lower limit of efficiency is given  
by additions of 0,05%, and it is preferable not to  
exceed the upper limit of 2%.

From their position in the electrochemical  
45 series antimony and bismuth are more valuable  
than magnesium, and moreover do not form a  
solid solution with the latter; the assumption  
therefore would rather have been that the addi-  
tion of these metals to the known alloys of mag-  
50 nesium would involve decreasing their resistance  
to corrosion.

The magnesium-base alloys developed by the  
present invention show also a considerable in-  
crease in strength, without the elongation de-  
55 creasing. As the magnesium alloys of the kind

hitherto in use (electron, Dow-metal) have a  
comparatively small strength, this constitutes a  
further advance of considerable importance, the  
more so as the specific gravity of the alloys is  
scarcely increased to any perceptible extent by 60  
the small amount of the added metals.

Furthermore, the alloys according to the invention  
show in comparison with similarly composed  
known electron alloys an increase of the perma-  
65 nent impact strength by 50%.

The alloys may be used as cast alloys or me-  
chanically worked alloys and may be improved by  
thermal treatments.

A satisfactory formula for an alloy according  
to my invention, in which zinc is the principal 70  
additional ingredient is as follows, viz:—

Magnesium 94,7%, zinc 4%, manganese 0,3%,  
antimony 1%;  
Magnesium 96,2%, zinc 3%, manganese 0,5%,  
75 bismuth 0,3%.

What I claim is:—

1. A low specific gravity magnesium-base alloy  
containing from about 80% to 98,8 per cent of  
magnesium, zinc in an amount between about 1  
per cent to about 20%, manganese in an amount 80  
of from about 0,12% to 2 per cent and subject to  
corrosion, this alloy being rendered more resist-  
ant against corrosion by the addition of at least  
one metal of the group consisting of antimony  
and bismuth in an amount from 0,05 to 2%. 85

2. A low specific gravity magnesium-base alloy  
consisting of from about 86% to 98,8% of mag-  
nesia, from about 1 to 10% of zinc, from about  
0,15 to 2% of manganese, and from about 0,05  
to 2% of at least one metal of the group consist- 90  
ing of antimony and bismuth.

3. A low specific gravity magnesium-base alloy  
consisting of from about 86 to 98,8% of mag-  
nesia, from about 1 to about 10% of zinc, from  
about 0,15 to 2% of manganese, and antimony 95  
and bismuth in a combined amount of from about  
0,05 to 2%.

GEORG SCHICHTEL.

100

105

110